

# UNITED STATES PATENT OFFICE.

WILLIAM B. OTWELL, OF CARLINVILLE, ILLINOIS, ASSIGNOR TO MINNESOTA LINSEED OIL PAINT COMPANY, OF MINNEAPOLIS, MINNESOTA, A CORPORATION.

## TREE-PAINT AND METHOD OF PREPARING SAME.

1,111,758.

Specification of Letters Patent. Patented Sept. 29, 1914.

No Drawing.

Application filed November 4, 1912. Serial No. 729,313.

To all whom it may concern:

Be it known that I, WILLIAM B. OTWELL, a citizen of the United States, residing at Carlinville, in the county of Macoupin and 5 State of Illinois, have invented certain new and useful Improvements in Tree-Paint and Methods of Preparing Same, of which the following is a specification.

My invention relates to a paint to be applied to fruit trees for the purpose of protecting the trunk of the tree from animals and insects.

It is the object of my invention to provide a paint for that purpose which may be put up at the factory in dry form and will keep after being put up until used without losing any of its efficacious properties. This dry paint is to be mixed with a requisite amount of water at the time of using and applied to 20 the trees, when a chemical action is set up between the ingredients of the paint so that the insecticide elements thereof will gradually be released in active form while at the same time the paint disintegrates upon the trunk 25 of the tree and will ultimately (in from four to six months time) be carried away to the roots of the trees where fertilizing constituents of the paint become available for plant food.

Nicotin is well known to be an extremely effective insecticide. All tobacco contains nicotin, and tobacco dust may be and is used quite generally for insecticide purposes. When, however, tobacco dust is mixed with 35 a liquid for application in the form of a paint the nicotin crystals are immediately released from the substance of the tobacco dust and washed away with the first rains, so that in the past tobacco dust has only been 40 effective by means of repeated applications for immediate results.

I have discovered that air slaked lime in combination with Venetian red may be made into a paint with tobacco dust, and after 45 the same has been applied and dried the lime and Venetian red will hold the nicotin in suspension in the body of the paint and prevent the rains from washing the same away except to the extent that the body of the 50 paint itself is washed away. It also operates to free the nicotin from the tobacco dust and will in time combine therewith. This freeing effect is gradual, however, and for that reason results satisfactorily when the paint

is applied to the tree, but for the same reason the tobacco dust and lime cannot be mixed even in dry form until ready for application upon the tree. It is an essential part of my invention that my complete compound is prepared dry in two separate parts 60 which are mixed together with the necessary quantity of water just before the same is applied to the tree. In practice, a sufficient amount of each of the sets of ingredients is prepared and packaged for mixing together 65 with a given quantity of water to produce a certain determined quantity of paint. The preferred proportions of ingredients for the mixture thereof containing tobacco dust is six parts by weight of powdered glue, six 70 parts by weight Venetian red, one part by weight flour of sulfur, and one part by weight powdered tobacco dust. All of these ingredients must be powdered very fine and intimately mixed together. Fourteen ounces 75 of this mixture will be required to make one gallon of the mixed paint.

The other set of ingredients comprises air slaked lime and Venetian red thoroughly pulverized and mixed together in the proportions of three parts of air slaked lime to one part of Venetian red. Five pounds two ounces of this mixture will be required for mixing a gallon of tree paint. In practice mixture number one, consisting of powdered 80 glue, flour of sulfur, Venetian red and powdered tobacco dust, in proportions stated, will be put up in packages of fourteen ounces or multiples thereof, and mixture number two, consisting of air slaked lime 85 and Venetian red, mixed in the proportions stated, will be put up in packages of five pounds two ounces or multiples thereof. These two packages of mixtures, numbers one and two, respectively, will be procured 90 by the user and mixed with a gallon of water in the orchard and immediately applied to the tree trunks. This paint should be applied early in the spring and may also be applied late in the fall. It will have entirely 95 washed away by the end of summer, and that applied in the fall will practically all be off of the tree trunks by the following spring, so that application should be made both spring and fall. It is essential that the 100 paint should wash off as indicated because if it does not do so and were to remain permanently upon the bark of the tree it would 105

both be injurious to the tree and fail to perform the insecticide functions for which it is primarily intended.

When used for winter I add to the paint 5 a mixture of coal tar and brown creosote in the proportions of one part by weight of coal tar and two parts by weight of brown creosote, and of this mixture add six ounces to each gallon of winter tree paint. The 10 mixture of tar and creosote will be shipped in sealed containers separate from the packages containing mixture number one and mixture number 2, and added to the paint in the orchard at the time of mixing.

15 I claim:

1. A tree paint consisting of glue, sulfur, tobacco dust, Venetian red, air slaked lime, water, coal tar and creosote intermingled and combined in the manner and approxi- 20 mately as specified.

2. The method of preparing a tree paint including tobacco dust as an insecticide, which comprises mixing together powdered glue, flour of sulfur, Venetian red and powdered 25 tobacco dust, separately mixing air slaked lime and Venetian red, separately packaging approximately fourteen ounces of mixture number one and approximately five pounds two ounces of mixture number two, and

mixing said sets of ingredients with water 30 immediately before using in the proportion of one gallon of water for each fourteen ounces of mixture number one and five pounds two ounces of mixture number two.

3. The method of preparing a tree paint 35 including tobacco dust as an insecticide which consists in mixing together powdered glue, flour of sulfur, Venetian red and powdered tobacco dust, separately mixing air slaked lime and Venetian red, separately 40 mixing coal tar and creosote, separately packaging approximately fourteen ounces of mixture number one, approximately five pounds two ounces of mixture number two, and approximately six ounces of mixture 45 number three, and mixing said sets of ingredients with water immediately before using in the proportion of one gallon of water for each fourteen ounces of mixture number one, five pounds two ounces of mix- 50 ture number two and six ounces of mixture number three.

In testimony whereof I affix my signature in presence of two witnesses.

1  
WILLIAM B. OTWELL.

Witnesses:

GERTRUDE DIXON,  
NETTIE JOHNSON.

Copies of this patent may be obtained for five cents each, by addressing the "Commissioner of Patents.  
Washington, D. C."